

## UNITED STATES PATENT OFFICE

2,305,673

## TREATMENT OF GASOLINE

Joseph A. Chenicek, Chicago, Ill., assignor to  
Universal Oil Products Company, Chicago, Ill.,  
a corporation of Delaware

No Drawing. Application February 29, 1940,  
Serial No. 321,572

15 Claims. (Cl. 44—72)

This invention relates to a method for improving the stability of hydrocarbon distillates insofar as color and gum formation are concerned. More particularly the process concerns improved methods of preventing deterioration of cracked gasolines which may be stored over relatively long periods of time in the presence of air.

The use of inhibitors to prevent the depreciation of olefin-containing hydrocarbon distillates such as cracked gasoline has been practiced. Such compounds as alkyl-substituted phenols, aminophenols, fractions of wood tar distillate, etc., have been added to cracked gasoline in relatively minor quantities, of the order of 0.001—0.1% to inhibit the formation of objectionable oxidation products and prevent loss of color and anti-knock properties of said gasolines during storage periods. The use of inhibitors has replaced or supplemented such forms of refining as acid-treating, clay-treating and the like. The result has been a material saving in refining costs as well as the conservation of substantial amounts of gasoline which were formerly lost in the refining steps.

The present invention offers a means of improving the inhibiting properties of gasoline inhibitors and of effecting material savings in the quantities of such material which may be required adequately to preserve the valuable properties of gasoline.

In one specific embodiment the present invention comprises a method for treating olefin-containing hydrocarbon distillates such as cracked gasoline to preserve the valuable properties thereof which consists in adding to said distillate a gasoline gum inhibitor together with a relatively minor quantity of hydroxy alkylene diamine.

These compounds have the general structural formula



wherein  $x$  and  $x'$  are integers. A representative compound is 1,3-diaminopropanol.

The present class of compounds are used in combination with recognized gasoline gum inhibitors such as N-substituted alkyl aminophenols, alkyl phenols, substituted phenol ethers, fractions of wood tar distillate boiling in the range of 240—280° C., and others. The compounds of this invention may be added to the gasoline separately or simultaneously with the gum in-

hibitor, or may be mixed with the gum inhibitor and the mixture added to the gasoline.

The quantity of hydroxyalkylene diamine commonly used in the gasoline is of the order of 0.0001—0.01% by weight thereof. The exact quantity required is a function of the inhibitor with which it is used and of the gasoline as well as the desired stability of the gasoline treated. The compounds of this invention are not of themselves gum inhibitors and the effect observed is not, therefore, the additive effect such as might be expected by the joint use of two gasoline gum inhibitors.

When the present types of compounds are added alone to cracked gasoline in amounts up to approximately 0.1%, little or no increase in the oxygen bomb induction period is to be observed and storage tests indicate that no protection is obtained for the gasoline under storage conditions. However, when used with an inhibitor, the induction period with a given quantity of the inhibitor is markedly increased and with the more effective compounds of this invention, more than equal weight percentages of the inhibitor can be replaced without suffering a loss in inhibitor potency. This will be brought out more fully in the example to be given later.

The compounds of this invention are not necessarily exactly equivalent in their effects and it should be understood that they cannot necessarily be used to replace one another in the composite inhibitor with equal effects either on a weight or a molal equivalent basis.

The following example is given to illustrate the usefulness and practicability of the process, but should not be construed as limiting it to the exact conditions or compounds given therein.

A Pennsylvania cracked gasoline was treated with a gasoline gum inhibitor comprising N-butyl aminophenol in concentrations of 0.01%. The gasoline thus treated had an oxygen bomb induction period of 330 minutes. When 0.01% of 1,3-diamino propanol was added to the inhibited gasoline, the induction period was 610 minutes. When the 1,3-diamino propanol was added to the gasoline without gum inhibitor present, the induction period was the same as that of the original uninhibited gasoline, namely 95 minutes.

I claim as my invention:

1. A process for treating olefin-containing hydrocarbon distillate to prevent depreciation thereof which comprises adding to said distillate a gasoline gum inhibitor and an hydroxy alkylene diamine.

2. A process for treating cracked gasoline to

prevent depreciation thereof which comprises adding to said gasoline a gasoline gum inhibitor and a compound of the following general structure:



wherein  $x$  is an integer.

3. A process for treating cracked gasoline to prevent depreciation thereof which comprises adding to said gasoline a gasoline gum inhibitor and a minor quantity of 1,3-diaminopropanol.

4. A process for treating cracked gasoline to prevent depreciation thereof which comprises adding thereto a gasoline gum inhibitor and an amount of an hydroxy alkylene diamine within the limits of approximately 0.0001-0.01% by weight of the gasoline.

5. A process for treating cracked gasoline to prevent depreciation thereof which comprises adding thereto a gasoline gum inhibitor in amounts of approximately 0.001-0.1% and an amount of an hydroxy alkylene diamine within the limits of approximately 0.0001-0.01%, both by weight of the gasoline.

6. A process for treating cracked gasoline to prevent depreciation thereof which comprises adding to said gasoline a gasoline gum inhibitor consisting of an N-substituted-alkyl aminophenol and an hydroxy alkylene diamine.

7. A process for treating cracked gasoline to prevent depreciation thereof which comprises adding to said gasoline a gasoline gum inhibitor consisting of a wood tar fraction boiling within the limits of approximately 240-280° C. and an hydroxy alkylene diamine.

8. An inhibitor for cracked gasoline compris-

ing essentially a mixture of a gasoline gum inhibitor and an hydroxy alkylene diamine.

9. An inhibitor for cracked gasoline which comprises essentially a mixture of a gasoline gum inhibitor and 1,3-diaminopropanol.

10. An inhibitor for cracked gasoline which comprises essentially a mixture of an N-substituted-alkyl aminophenol with an hydroxy alkylene diamine.

11. An inhibitor for cracked gasoline which comprises essentially a mixture of a wood tar distillate boiling within the limits of approximately 240-280° C. and an hydroxy alkylene diamine.

12. A composition of matter useful for inhibiting the oxidation of unstable organic substances such as olefin-containing hydrocarbon distillates which comprises a mixture of an antioxidant with an hydroxy alkylene diamine.

13. A composition of matter useful for preventing the oxidation of unstable organic substances which comprises a mixture of an antioxidant with 1,3-diamino propanol.

14. In the art of stabilizing olefinic distillates against deterioration by the addition of gum inhibitors thereto, the method of increasing the gum inhibiting potency of the inhibitor which comprises incorporating into the olefinic distillate, in addition to the gum inhibitor, a relatively small amount of a hydroxy alkylene diamine.

15. A stabilizing agent suitable for retarding gum formation in olefinic distillates comprising a phenolic gum inhibitor and an amount of a hydroxy alkylene diamine such as to increase the inhibiting potency of the phenolic inhibitor.

JOSEPH A. CHENICEK.